

# UNITED STATES PATENT OFFICE.

WARREN K. LEWIS, OF NEWTON, MASSACHUSETTS, ASSIGNOR TO THE GOODYEAR  
TIRE & RUBBER COMPANY, OF AKRON, OHIO, A CORPORATION OF OHIO.

## PREPARATION OF LAMPBLACK.

1,418,811.

Specification of Letters Patent. Patented June 6, 1922.

No Drawing.

Application filed August 13, 1918. Serial No. 249,640.

To all whom it may concern:

Be it known that I, WARREN K. LEWIS, a citizen of the United States, residing at Newton, in the county of Middlesex and State of Massachusetts, have invented a new and useful Improvement in the Preparation of Lampblack, of which the following is a specification.

My invention relates to the art of preparing lamp black or carbon black and will be fully understood from the following specification:

Practically all of the carbon black or lamp black of commerce is now prepared by burning natural gas or other hydrocarbon or related carbonaceous fuel with an insufficient supply of air, the flame being chilled by impinging upon a relatively cool place which will serve as the surface on which the free carbon resulting from the imperfect combustion is deposited. The actual yield of lamp black by this process is relatively low as compared with the mass of carbon in the fuel burned, and it is further well recognized that for the production of lamp black of the highest grade suitable for paints having great covering power, the yield must be kept well below the maximum yield obtainable by the ordinary process. I have discovered that it is possible to largely increase the yield of carbon black now obtained in the combustion of, for example, a hydrocarbon gas and at the same time effect an improvement in the quality of the carbon black from the standpoint of fineness or covering power, by a modification of the conditions under which the actual combination occurs. In its broadest aspect, such modification consists in causing the combustion to take place in what may be described as a dilute gaseous solution of hydrocarbon and oxygen, that is, instead of admixing with the natural gas oxygen and nitrogen in the proportions existing in the atmosphere, the percentage of oxygen being somewhat less than that required for complete combustion of the natural gas, there should be present a relatively large diluting volume of an inert gas such, for example, as combustion gases obtained from the combustion of natural gas, or any other carbona-

ceous hydrocarbon fuel. This diluting inert gas should preferably be admixed both with the natural gas and with the air, in order to insure a completely homogeneous atmosphere in which the combustion takes place.

Under these conditions, the individual hydrocarbon molecules are separated by a considerable distance at the time combustion or partial combustion takes place. By reason of this separation the number of contacts between the nascent carbon molecules is proportionately reduced with a resultant reduction in the size of the aggregates or particles which are eventually formed either before or in the act of deposition upon a cool surface. The dilution has a further beneficial effect in that there is present a relatively large envelop of the diluting inert gas around each hydrocarbon molecule, this envelop serving as a heat absorber which rapidly reduces the temperature of the combustion products including the carbon. Such reduction in flame temperature, accomplished within the body of the flame itself by the diluting atmosphere, should, in accordance with the kinetic theory of gases, also reduce the mean velocity of the nascent carbon molecules and by proportionately reducing the number of contacts between molecules, retard formation of aggregates.

The beneficial effects of my improvement in the art are not qualitative alone but also quantitative, i. e., it is possible by the practice of the invention to increase the yield of carbon black per cubic foot of gas consumed. This result in part follows from the improvement in quality for, as heretofore stated, it is well known that the yield of carbon black may be increased considerably if the quality, i. e., degree of fineness, be sacrificed. Since fineness of the product according to my process is assured by principles other than percentage of oxygen supplied to the natural gas, it follows that, as compared with the old or known processes, it is possible to obtain a greater yield of black of the same quality or grade of fineness as that produced by the known expedient of reducing the percentage of oxygen with reference to the hydrocarbon. This result of increased yield may be expected to be still further

benefited, however, by the use of combustion gases as a diluent because of their containing a high percentage of carbon dioxide. Considered from the standpoint of the equilibrium or mass reaction theory, or from the standpoint of the tendency of that reaction to take place which will liberate the greatest amount of heat (which principle has in recent years been modified as involving the taking place of that reaction which results in the greatest degradation of energy), or from the standpoint of the relative affinities of hydrogen and carbon for oxygen, the presence of carbon dioxide in considerable

proportions in the atmosphere in which the combustion takes place, must inevitably result in the combustion of a smaller proportion of the carbon of the hydrocarbon. The degree to which this effect is obtainable is dependent to a large extent upon the flame temperature but, for the reasons stated, the employment of combustion gas or other carbon-dioxide containing gas as a diluting atmosphere, is preferred.

As is suggested in the foregoing, the extent to which dilution may be carried out is limited by the flame temperature or the minimum temperature at which flame propagation takes place. As a specific example of one method of carrying out my invention to produce a high yield of carbon black of a grade equal to or better than that now produced by the ordinary methods, the following may be given:

The natural gas is diluted with 4 to 5 volumes of combustion gas, which may be the gas obtained from the combustion of the natural gas itself in the process of manufacturing carbon black, or may be obtained from any other source, and the air supply before admission to the combustion chamber is likewise diluted with 1 to 2 volumes of combustion gas. Since natural gas requires approximately ten times its own volume of air for combustion, the total quantity of diluting combustion gas may be from 14 to 25 times the volume of natural gas. Thus the total proportional quantity of diluting combustion gas may be, in the preferred process, from 15 to 20 volumes, based on the volume of natural gas. One of the major advantages accruing from this invention is the flexibility in control of plant operations which results therefrom. By variation of the amount of diluent gas employed, combined with variation in temperature and amount of cooling water and the like, it is possible either to secure a much larger yield of black of a quality equal to that at present obtained without sacrificing the yield, or to combine these two advantages. This makes possible wide modification of factory product to meet market conditions without change in plant design.

While I have described in considerable

detail what I believe to be the principles underlying and mechanism of my process, and have given one specific example of the method of carrying out the process, it will be understood that my invention is not dependent upon the soundness or accuracy of the theories which I have advanced, nor limited to the exact process disclosed, except in so far as such limitations are included within the terms of the accompanying claims, in which it is my intention to claim all novelty inherent in my invention as broadly as is permissible in view of the prior art.

What I claim is:

1. The improvement in the art of producing carbon black by the imperfect combustion of hydrocarbons which comprises in admixing said hydrocarbons prior to combustion with a relatively large proportion of inert gas sufficient to reduce the carbon content thereof to a fraction of that of natural gas.

2. The improvement in the art of producing carbon black by the imperfect combustion of hydrocarbons which comprises in admixing said hydrocarbons prior to combustion with a relatively large proportion of diluting gas containing an oxide of carbon sufficient to reduce the carbon content thereof to a fraction of natural gas.

3. The improvement in the art of producing carbon black by the imperfect combustion of hydrocarbons which comprises in admixing said hydrocarbons prior to combustion with a relatively large proportion of combustion gas sufficient to reduce the carbon content thereof to a fraction of that of natural gas.

4. The improvement in the art of producing carbon black by the imperfect combustion of carbonaceous compounds, which comprises in admixing with the air used for combustion a relatively large proportion of inert gas.

5. The improvement in the art of producing carbon black by the imperfect combustion of carbonaceous compounds, which comprises in admixing with the air used for combustion a relatively large proportion of inert diluting gas containing an oxide of carbon.

6. The improvement in the art of producing carbon black by the imperfect combustion of natural gas, which comprises in admixing with the air used for combustion a relatively large proportion of combustion gas.

7. The improvement in the art of producing carbon black by the imperfect combustion of carbonaceous compounds, which consists in causing such combustion to take place in the presence of approximately 15-20 volumes of inert diluting gas.

8. The improvement in the art of producing carbon black by the imperfect combustion of carbonaceous compounds, which con-

sists in causing such combustion to take place in the presence of approximately 15-20 volumes of diluting gas containing an oxide of carbon.

5 9. The improvement in the art of producing carbon black by the imperfect combustion of natural gas, which consists in caus-

ing such combustion to take place in the presence of approximately 15-20 volumes of combustion gas.

WARREN K. LEWIS.

Witnesses:

R. S. TROGNER,  
E. C. LEADENHAM.